

P. M. STEWART.  
PROTECTED METAL ARTICLE.  
APPLICATION FILED DEC. 13, 1916.

1,236,994.

Patented Aug. 14, 1917.

*Fig. 1.*



*Fig. 2.*



*Invantor*  
Perez M. Stewart  
by Jas. H. Churchill  
atty.

# UNITED STATES PATENT OFFICE.

PEREZ M. STEWART, OF NEW YORK, N. Y., ASSIGNEE TO GERTRUDE F. STEWART, OF NEW YORK, N. Y.

## PROTECTED METAL ARTICLE.

1,236,994.

Specification of Letters Patent. Patented Aug. 14, 1917.

Application filed December 13, 1916. Serial No. 136,775.

To all whom it may concern:

Be it known that I, PEREZ M. STEWART, a citizen of the United States, and a resident of the borough of Manhattan, in the city, county, and State of New York, have invented an Improvement in Protected Metal Articles, of which the following description, in connection with the accompanying drawings, is a specification, like characters 10 on the drawings representing like parts.

This invention relates to a protected metal article especially adapted among other uses to be employed for building purposes.

The invention has for its object to provide 15 a metal article with a protective layer of fibrous material, such as asbestos paper, felt and the like, which is adhesively secured to the metal article in a superior manner and by means of an adhesive which in itself forms 20 a firm, tough and highly efficient protective layer for the metal member.

The fibrous layer may and preferably will be provided with a surface coating which is hard, tough, and a superior resistant to 25 abrasion, weather and acid and alkali fumes.

To this end, the metal article is provided with a coating or layer of polymerizable material, such as Chinese wood oil, and while the coating is still tacky, a layer of fibrous 30 material, such as asbestos paper, felt and the like, is applied to the coated metal article and in turn has applied to it a layer of polymerizable material, and the article thus protected is subjected to heat to bake the layers 35 of the polymerizable material.

These and other features of this invention will be pointed out in the claims at the end of this specification.

Figure 1 is a plan view of a metal article 40 embodying this invention, and

Fig. 2, a section on the line 2—2, Fig. 1.

Referring to the drawing, *a* represents a metal article, which is shown in sheet form and preferably of steel.

45 The steel sheet *a* has applied to it a coating or layer *b* of polymerizable material, preferably Chinese wood oil alone or mixed with other materials, and is further provided with a layer *c* of fibrous material, such as asbestos paper, felt or the like, which in turn has applied to it a layer or coating *d* of polymerizable material, such as Chinese wood oil alone or mixed with other materials, such as resins, asphalt, coal tar and its 50 derivatives.

The protected metal article thus produced is subjected to heat to bake the polymerizable layers, which are rendered firm, tough and resistant to abrasion, weather, and acid and alkali fumes, thereby rendering the protected metal article especially useful for 60 building purposes.

The metal article *a* may be coated with the polymerizable layer *b* by passing the metal article through a bath of the polymerizable 65 material, and while the latter is in an adhesive condition, the fibrous layer *c* is applied to the metal article so as to cover the same and preferably so as to envelop the metal article and seal the edges of the latter, and the exterior layer *d* of polymerizable material may be applied by hand or machinery or in any other suitable manner, after which the protected article is subjected 70 to heat in a suitable oven or room to bake the 75 external layer of polymerizable material and preferably also the internal layer which adheres to the metal article.

It is preferred to heat the protected metal article a sufficient length of time to bake the 80 internal layer of polymerizable material as by so doing the said layer is rendered firm, hard and tough, in which case the metal article is sealed and protected from corrosion.

Furthermore the fibrous layer is secured 85 to the metal article in a superior manner, as the internal layer of polymerizable material penetrates more or less into the inner or under surface of the fibrous layer, so that when the internal polymerizable layer is baked, it 90 hardens within the fibrous layer as well as on the steel or other metal article and secures the fibrous layer to the metal article in a firm and superior manner.

The external layer of polymerizable material when baked forms a firm, tough and hard wearing surface, which resists abrasion, and enables the article to be handled in transportation and on the job with less liability of being injured so as to expose the 95 metal member to extraneous detrimental influences.

It also forms a surface which resists the weather and also acid and alkali fumes.

As a result a superior protected metal article is produced, which is especially adapted 100 for use for building purposes.

I have herein represented the metal article as a sheet, but it is not desired to limit 110 the invention in this respect, as it may be of

any desired form, as, for instance, an I or T beam, channel bar, angle iron, and the like.

It is preferred to use both the internal and external layers of polymerizable material, 5 but it is not desired to limit the invention in this respect, as either alone may be used to advantage.

Claims.

1. A protected metal article comprising a 10 metal member provided with a coating of baked polymerizable material, a fibrous layer affixed to the metal member by said polymerizable material, and a layer of baked polymerizable material on the exterior surface 15 of said fibrous layer.

2. A protected metal article comprising a metal member provided with a coating of baked polymerizable material, and a fibrous

layer affixed to said metal member by said baked polymerizable material. 20

3. A protected metal article comprising a metal member provided with a layer of baked Chinese wood oil, and a layer of asbestos affixed to the metal member by said baked layer. 25

4. A protected metal article comprising a metal member provided with a layer of baked Chinese wood oil, a layer of asbestos affixed to the metal member by said baked layer, and a layer of baked Chinese 30 wood oil on the exterior surface of said asbestos layer.

In testimony whereof I have signed my name to this specification.

PEREZ M. STEWART.